

## 1

3,121,765

### PROCESS FOR THE MANUFACTURE OF ACRYLIC SYNTHETIC FIBER

Ichiro Kanda, Michiaki Nakajima, and Makoto Amiya, all of Kitajima-machi, Itano-gun, Tokushima Prefecture, Japan, assignors to Toho Rayon Kabushiki Kaisha, Tokyo, Japan, a corporation of Japan  
No Drawing. Filed Sept. 18, 1961, Ser. No. 138,581  
Claims priority, application Japan Sept. 24, 1960  
4 Claims. (Cl. 264—182)

This invention relates to a process for the manufacture of a synthetic acrylic fiber by spinning a spinning solution comprising zinc chloride solution and polymer containing acrylonitrile as a principal constituent, and then treating the coagulated tow with an aqueous solution of a compound so as to produce a zinc complex ion with the object of avoiding the degradation of fiber quality due to remaining salts.

It has been reported that in fiber products obtained from an acrylic polymer solution using concentrated aqueous inorganic salt solution containing zinc chloride as a principal constituent, inorganic salts particularly zinc compound in the form of hydroxide or oxide remained in the fibers and that such residual salts caused the quality of the products to be unfavorably reduced. For instance, fiber containing a residual salt of more than 1 percent by weight is brittle and dyed in dull color, and upon heating it becomes yellowish and weak. To improve on the above disadvantages, it has been proposed to apply an ion-exchange resin method of Japanese Pat. Publn. No. 2,369/56, or a zinc chloride method by treating the fiber with compounds such as sodium ethylenediamine tetraacetate according to the Japanese Pat. Publn. No. 8,444/57. But these methods are too expensive for industrial practice.

The present invention has been reached by our new knowledge on the effect of compounds, forming complex ion with zinc ion, such as ammonium, amine or chlorine, and the process is industrially useful and practicable.

Desalting agents, in the present invention, are sodium chloride, potassium chloride, ammonium chloride, urea, thiourea and others, that is, electron donor compounds which coordinate to cation forming complex ion. These compounds which have chloride, ammonium ion, or amino group can form complex ions with the zinc ion as in the following. Halides, such as NaCl, KCl, NH<sub>4</sub>Cl form complex ions, some of which are [ZnCl<sub>4</sub>]<sup>2-</sup> and [ZnCl<sub>3</sub>OH<sub>2</sub>]<sup>-</sup>, and in the case of NH<sub>4</sub>Cl occur, moreover, amine complexes, such as



and so on. In the case of urea and thiourea occur [Zn(NH<sub>2</sub>CONH<sub>2</sub>)<sub>4</sub>]<sup>2+</sup> and [Zn(NH<sub>2</sub>CSNH<sub>2</sub>)<sub>4</sub>]<sup>2+</sup> respectively. All of these complex ions have tetrahedral 4-coordinated structure.

The salt removal treatment based on the above discovery may be applied to a dried fiber, but from the point of easiness in removing the salt and of simplification in industrial fiber process, it is effected during or after the washing process of coagulated tow with water which has been coagulated from a spinning solution as is a common practice, and then the coagulated tow is treated with an aqueous solution of above mentioned compounds.

According to this invention, by immersing tow after being passed through the coagulating bath in an aqueous solution of desalting agents, zinc compounds, which remained in the tow as hydroxide or hydrated oxide of zinc, can diffuse and dissolve out into the solution as water soluble complex ions.

The tow which is formed by extruding a polymer solu-

## 2

tion into a coagulating bath comprised of a more dilute aqueous salt solution of the same or similar salt system as employed in the solvent of the polymer solution, may be stretched at moderate temperature in water, or stretched under moderate temperature and humidity after water washing. Thereafter, it may go through required aftertreatments, such as oiling, heat stretching and relaxing processes that are in common practice.

The salt removing treatment is accomplished, according to this invention, by using 1 to 20 percent aqueous solution of desalting agent, preferably 5 to 15 percent, at 70° C. to boiling temperature, preferably over 90° C.

Results according to a few examples of salt removal treatment are shown in the following Table 1, using coagulated tow B in the following Example 1. Tow B is composed of 52.6% polymer, 45.1% water and 2.3% zinc chloride, and, when squeezed and dried in air, it contains 0.39% residual zinc.

The tow B treated with various salt removal treatments (I, II, III, IV and V) and dried in air to 1 percent moisture content was analyzed and found to include residual zinc chloride as follows:

TABLE 1

| Method                               | I     | II    | III   | IV    | V     |
|--------------------------------------|-------|-------|-------|-------|-------|
| Residual ZnCl <sub>2</sub> , Percent | 0.173 | 0.150 | 0.024 | 0.026 | 0.029 |

I. Several repeats of washing by boiling water for 30 minutes.  
II. Immersing for 24 hours in running water at room temperature.  
III. Immersing in 5% NH<sub>4</sub>Cl aqueous solution (see example).  
IV. Immersing in boiling 7% NaCl aqueous solution for 2 minutes and washing with water.  
V. Using 10% urea aqueous solution similarly to (IV).

35 Salt removal, according to the present invention, inexpensively and in a simple manner attains superior results as shown in the table above.

The following examples illustrate the practices of this invention, but are not to be construed as limiting.

#### Example 1

A solution was prepared consisting of 9% by weight of copolymer containing 95 mole percent of acrylonitrile and 5 mole percent of methyl acrylate having a Staudinger molecular weight of 82,000, 50.9% by weight of zinc chloride and 41% of water. This solution, having a viscosity of 360 poises at 30° C., was extruded through a 100-hole spinneret having openings respectively 0.08 mm. in diameter, into an aqueous solution of 15% by weight of zinc chloride at 15° C. The so-coagulated tow of filament was stretched 1.6 times its original length during washing with water (the sample here called A), and then stretched in boiling water three times its cold stretched length (sample B). This tow B of stretched fibers was washed with water and, when dried in air to 1% moisture content, had 0.39% of zinc chloride. This tow was boiled in an aqueous solution of 5% by weight of ammonium chloride for 2 minutes, then washed with water and, when dried, had 0.024% of zinc chloride.

#### Example 2

The tow A in Example 1 was stretched in boiling water containing 7% of sodium chloride two times its original length and then in boiling water 5 times its original length, and when dried, had only 0.034% of zinc chloride in it.

#### Example 3

The other portion of tow A was treated with aqueous solution of 10% of urea, washed with water and, when dried, had 0.039% of zinc chloride. The other portion of tow B was treated similarly as A and had had only 0.029% of zinc chloride.

What we claim is:

1. A method for manufacturing acrylic synthetic fibers comprising spinning into a coagulated tow a solution of a polymer containing acrylonitrile and a solvent of aqueous zinc chloride, contacting the coagulated tow with an aqueous solution containing 1 to 20 percent of a desalting agent chosen from the group consisting of ammonium chloride, sodium chloride, potassium chloride, urea and thiourea, and maintaining the aqueous solution in a temperature range of from 70° to 100° C.

2. The method as recited in claim 1, wherein the aqueous solution contains 5 to 15 percent of the desalting agent.

3. A method for manufacturing acrylic synthetic fibers comprising spinning into a coagulated tow a solution of a polymer containing acrylonitrile and a solvent of aqueous zinc chloride, contacting the coagulated tow with an aqueous solution containing 1 to 20 percent of a desalt-

ing agent chosen from the group consisting of ammonium chloride, sodium chloride, potassium chloride, urea and thiourea, and maintaining the aqueous solution in a temperature range of from 90° to 100° C.

4. The method as recited in claim 3, wherein the aqueous solution contains 5 to 15 percent of the desalting agent.

References Cited in the file of this patent

10

UNITED STATES PATENTS

|           |           |       |               |
|-----------|-----------|-------|---------------|
| 2,558,730 | Cresswell | ----- | July 3, 1951  |
| 2,558,781 | Pollard   | ----- | July 3, 1951  |
| 2,648,592 | Stanton   | ----- | Aug. 11, 1953 |

FOREIGN PATENTS

|         |               |       |              |
|---------|---------------|-------|--------------|
| 564,327 | Canada        | ----- | Oct. 7, 1958 |
| 636,476 | Great Britain | ----- | May 3, 1950  |